

# United States Patent [19]

Mead et al.

[11] 4,140,618

[45] Feb. 20, 1979

[54] TRANSFORMER OIL PROCESSING

|           |         |                   |         |
|-----------|---------|-------------------|---------|
| 2,370,228 | 2/1945  | Bruun et al. .... | 208/3   |
| 3,124,622 | 3/1964  | Cywinski ....     | 260/682 |
| 3,223,615 | 12/1965 | Magee ....        | 208/3   |
| 3,725,253 | 4/1973  | Yaznada ....      | 208/3   |

[75] Inventors: **Theodore C. Mead**, Port Neches;  
**Norman R. Odell**, Nederland, both of  
Tex.

[73] Assignee: **Texaco Inc.**, New York, N.Y.

[21] Appl. No.: **811,334**

[22] Filed: **Jun. 29, 1977**

[51] Int. Cl.<sup>2</sup> .. **C10G 34/00**

[52] U.S. Cl. .... **208/3; 208/14;**  
..... **208/211**

[58] Field of Search ..... **208/3, 14, 211**

## [56] References Cited

### U.S. PATENT DOCUMENTS

1,988,731 1/1935 Haslam ..... 208/85

*Primary Examiner*—Herbert Levine

*Attorney, Agent, or Firm*—Carl G. Ries; Thomas H.  
Whaley; Kenneth R. Priem

## [57] ABSTRACT

A transformer oil processing sequence is disclosed. The process comprises contacting a naphthenic based oil with an oxygen-containing gas in the presence of a free radical initiating catalyst under mild oxidation conditions of temperature and pressure, fractionally distilling the resultant product and then hydrogenating the oil.

12 Claims, No Drawings

## TRANSFORMER OIL PROCESSING

### BACKGROUND OF THE INVENTION

#### Field of the Invention

This invention pertains to the field of processing transformer oils.

This invention relates to mineral oils used as electrical insulating oils as in transformer switches and the like and generally called transformer oils. More particularly, it relates to the use of a particular processing sequence beginning with the preoxidation of the mineral oil under very mild conditions of temperature and pressure before further processing steps.

Oils used as electrical insulating oils in transformers or switches must be capable of resisting current conduction at voltage levels much higher than the voltages at which a transformer switch is normally operated since severe surges of voltage can occur in transformers and switches exposed to systemic disturbances such as lightning. This property of an insulating oil is termed its impulse strength. In addition, these oils must have an inherent resistance to oxidative processes which break down such oils and make them unfit for their intended purpose. With additive oxidation inhibitors they should show a substantial increase in oxidative resistance over their inherent oxidative resistance.

Heretofore insulating oils with acceptable properties have been produced by various methods which usually included sulfuric acid treating. However, sulfuric acid treating is not preferred since it produces large amounts of sludge which must be disposed of. Environmental considerations demand that processes be developed which eliminate this sludge problem. In the present invention, a catalyzed preoxidation step is used which when used in combination with the other steps produces an oil having superior properties necessary for insulating oils. U.S. Pat. No. 3,725,253 discloses a process for the purification of lubricating oils which comprises first reacting the mineral oil with an oxygen-containing gas catalytically at temperatures ranging from 108° C. to 280° C. This severe process results in the destruction of a large percentage of the incoming charge stock and consequent massive sludge formation. The process of the patent is completely different from the process of the present invention since the preoxidation step in the present invention is carried out at a much lower temperature resulting in almost no impurity generation. Thus, it is clear that the patent is directed to a completely different process which has as its aim a completely different objective and achieves different results than this invention.

U.S. Pat. No. 3,105,812 describes a process for removing nitrogen-containing compounds from cracking and hydrocracking feed stocks by catalytic oxidation followed by hydrogenation. The oxidation is catalyzed by phosphorous oxide or a phosphorous oxide and vanadium oxide mixture. As the patent points out, the vanadium oxide catalyst, which is a relatively well known oxidation catalyst, is not very effective used alone. Although the claims of the patent include a temperature between 100 and 600° F. for the oxidation step, the examples given in the patent were carried out at from 300 to 400° F. It has been found in using the process of our invention that oxidation of transformer oil stocks can be carried out at a much lower temperature routinely. This is surprising in view of the data in U.S. Pat. No. 3,105,812. At column 10, lines 51-59 the patent

teaches that a charge stock boiling in the range of a typical transformer oil distillate (550-750° F.) is best hydrogenated at 800-1600 psi. Using the process of our invention, the hydrogenation pressure is much lower.

5 The invention to be disclosed below uses a unique catalyst system for preoxidizing a transformer oil feed stock at very mild conditions. The fact that this can be done is surprising from the prior art which teaches oxidation of hydrocarbon oil feed stocks at much more severe conditions. The mild conditions to be delineated below have very real advantages in fuel savings, required metallurgy, and capital investments as well as other considerations.

#### SUMMARY OF THE INVENTION

The invention comprises first treating a suitable naphthenic transformer oil charge stock by catalytic oxidation at a temperature below about 275° F. and at pressure ranging up to about 300 psi in the presence of a free radical initiating catalyst, second, fractionally distilling the product and thirdly, contacting the overhead with hydrogen in the presence of a hydrogenation catalyst at a temperature of from about 400 to 675° F. and at a pressure from about 15 to 400 psi at a space velocity ranging from 0.1 to 10.0 vol/vol/hr.

#### DESCRIPTION OF THE PREFERRED EMBODIMENTS

30 Examples of suitable hydrocarbon oil charge stocks for the process of this invention are those naphthenic distillates which typically boil in the range of 250 to 400° C. and have viscosities in the range of 40 to 100 SUS, preferably 50 to 60 SUS at 100° F. It is also possible to obtain transformer oils from distillates with viscosities as low as 30 and as high as 150 SUS at 100° F. The transformer oil stocks are initially obtained from the distillation of crude naphthenic petroleum. The stock may be obtained as overhead from a vacuum distillation or may be obtained from the residue of vacuum distillation by deasphalting the residue by contact, for example, with a deasphalting agent such as propane, butane and the like or mixtures thereof.

#### Preoxidation

50 There are present in unprocessed lubricating oils molecular structural types which are particularly susceptible to oxidation and thermal and chemical degradation. These types include olefins, nitrogenous compounds, other compounds containing heteroatoms, certain types of aromatics and others. If allowed to remain in transformer oils, oxidation products of these species are polar or acidic in nature and tend to degrade the electrical insulating properties of transformer oils. Sulfuric acid treating has in the past removed such oxidizable species. This invention will show that other vigorously oxidizing conditions, not involving the use of sulfuric acid, can oxidize susceptible molecular types. The oxidates thus formed can then be removed or rendered innocuous by other processing steps to be pointed out herebelow.

55 The oxidation step is carried out catalytically with any common free radical initiating catalyst. Operable concentration range of the catalyst is from 0.0001 to 0.1 weight percent basis oil. Free radical initiating catalysts useful in this invention include alkyl, cycloalkyl or aryl hydroperoxides or peroxides. Also azo- type initiators are useful as free radical initiating catalysts.

In a preferred embodiment the catalyst system also includes potassium fluoride in addition to the free radical initiating catalyst mentioned above.

The temperature at which the oxidation step should be performed is from ambient temperature to 275° F. The preferred range is from 150 to 275° F. This temperature may vary depending on the rate at which air is fed into the reactant mixture. However, the oxidation temperature is a function of the exothermic temperature of the reaction and generally does not require external heating. It is preferred to adjust the air dosage rates so that the heat generated by the oxidation is just sufficient to maintain the required mild reaction temperature.

The operable pressure for the oxidation reaction is up to about 300 psi. It is preferred to operate at about atmospheric pressure if possible. The dosage rate of oxidizing gas (oxygen) is from about 0.01 to 5.0 SCF per minute per kilogram of oil. However, this dosage rate will depend on the concentration of inert diluent in the oxidizing gas, and the desired operating temperature as well as other operating variables. It is preferred to use from about 0.01 to 3.0 SCF per minute per kilogram of oil when possible.

The oxidizing gas may be chosen from the group consisting of air, oxygen, ozone, oxides of nitrogen and combinations of these with addition of inert diluents such as nitrogen. It is preferred to use air and oxygen-nitrogen mixtures whenever possible.

#### Fractional Distillation

After the oxidation step the oil is fractionally distilled. The percentage of overhead taken may vary between 50 and 99 percent.

#### Hydrogenation

Catalytic hydrogenation (hydrorefining) is performed at a temperature between about 400 to 675° F., preferentially between about 550 to 600° F. under a hydrogen pressure between about 15 to 400 psi preferably between about 300 and 350 psi, utilizing an hourly space velocity (v/v/hr) of between about 0.1 to 10 volumes of oil per volume of catalysts per hour, prefera-

VIII metals or compounds thereof such as the oxides or sulfides. Examples of Group VIII metals which may be used in the hydrogenating compound are nickel, cobalt or iron or mixtures thereof. The Group VIII metal should be present in an amount between about 2 and 10 weight percent, preferably between about 5 and 6 weight percent calculated as metal oxide based on the total weight of the catalyst composite. In conjunction with the Group VIII metal, a Group VI metal such as molybdenum or tungsten may be used. In such case, the Group VI metal may be present in an amount between about 10 and 30 weight percent based on the weight of the composite, a preferred range being about 12 and 15 weight percent.

5 The hydrogenating catalyst component is carried on a base comprising a refractory inorganic oxide material such as alumina, silica, magnesia, zirconia, titania, crystalline alumino silicates and the like, and mixtures thereof.

#### EXPERIMENTAL

A 55 second (at 100° F.) naphthene pale stock (68.1 pounds), free radical initiator catalyst azobisisobutyronitrile (AIBN; 5 g) and potassium fluoride (5 g) were aerated at 2 SCFM of air for six hours at 250° F. Oxidate had a neutralization number of 1.1 at the conclusion of air blowing. The oil was agitated with 400 ml 15° Be caustic for thirty minutes with nitrogen; it was then water washed until free of caustic and brightened at 180° F. by purging with nitrogen at 2 SCFM.

25 Caustic-washed and brightened oxidate was distilled at 10 mm pressure until 90.44 wt% was obtained as overhead. Overhead temperature at the completion of the distillation (corrected to 760 mm) was 727° F.

30 Overhead from this distillation was hydrogenated at 610° F., 340 psi hydrogen pressure at a LHSV of 0.6 volumes of oil per volume of catalyst per hour. A dosage of 500 SCFB of hydrogen was used; American Cyanamid HDS-3A nickel-molybdenum on alumina catalyst was employed.

35 Hydrogenated oil was subjected to electrical insulation testing as recorded in the table below.

#### PERFORMANCE OF OXIDIZED-DISTILLED-HYDROGENATED TRANSFORMER OIL

| Test                                                     | ASTM-D | Typical Commercial Product | Product Performance |              |
|----------------------------------------------------------|--------|----------------------------|---------------------|--------------|
| Neutralization number                                    | 974    | 0.02                       | max                 | 0.10 (0.02)  |
| Dielectric strength, kv                                  | 877    | 30                         | min                 | 40 40        |
| Dielectric strength, kv                                  | 1816   | 20                         | min                 | 24 24        |
| Power factor, 60 cycles<br>25° C., 10 v/mil              | 924    |                            |                     |              |
| 100° C., 10 v/mil                                        |        | 0.05                       | max                 | 0.01 (0.05)* |
| Resistivity, ohm-cm<br>25° C., 10 v/mil $\times 10^{12}$ | 1169   | 0.03                       | max                 | 0.06 (0.11)* |
| 100° C., 5 v/mil $\times 10^{12}$                        |        |                            |                     |              |
| Dobie                                                    |        |                            |                     |              |
| Power factor valued oxidation, hr                        |        | 70                         | min                 | 881 881      |
| Sludge free life, hr                                     |        | 30                         | min                 | 132 (13)*    |
|                                                          |        |                            | 21                  | (1)*         |
|                                                          |        |                            | 96                  | (24)*        |

\*Values obtained from oxidized-hydrogenated (but not distilled) product.

bly between about 0.5 to 1.5 vol/vol/hr with a hydrogen dosage of between about 50 and 500 standard cubic feet per barrel (scfb), preferably between about 200 and 400 scfb. The hydrogen gas used for the hydrogenation step need not necessarily be a pure hydrogen. Hydrogen having a purity of at least about 65 volume percent preferably about 75 volume percent may be employed.

The catalyst employed in the hydrogenation step generally comprises a hydrogenation component on a support. The principal ingredient of the hydrogenation component is a Group VIII metal or mixtures of Group

60 Employing the method of U.S. Pat. No. 3,749,666 in which the oxidation was carried out at 250° F. in the presence of 2.5 wt% sulfuric acid resulted in the formation of 7 pounds of acid sludge from 136.2 pounds of 55 second naphthenic distillate charge. In the method of this invention (as shown above) the same charge was oxidized unexpectedly, without measurable sludge formation.

We claim:

1. A method of making transformer oils comprising

(a) contacting a napthenic oil with an oxygen-containing gas in the presence of a catalyst system comprising a free radical initiating catalyst at a temperature below 275° F. and a pressure ranging up to 300 psi,

(b) fractionally distilling the product of (a), and  
(c) contacting the overhead from (b) with hydrogen

in the presence of a hydrogenation catalyst at a temperature of from about 400 to 650° F. and at a pressure of about 15 to 400 psi at a space velocity ranging from 0.1 to 10.0 vol/vol/hr at a hydrogen dosage between about 50 and 500 scfb.

2. A method as in claim 1 wherein the oxygen-containing gas is air. 15

3. A method as in claim 1 wherein the free radical initiating catalyst in step (a) is selected from the group consisting of alkyl, cycloalkyl and aryl hydroperoxides or peroxides and azo- type compounds. 20

4. A method as in claim 3 wherein the catalyst system also includes potassium flouride.

5. A method as in claim 1 wherein the catalyst system comprises azobisiso-butyronitrile and potassium fluoride. 25

6. A method as in claim 1 wherein the temperature in step (a) is from about 150 to 275° F.

7. A method as in claim 1 wherein the temperature in step (c) is from about 550 to 600° F.

8. A method as in claim 1 wherein the oxygen-containing gas is air.

9. A method as in claim 1 wherein the pressure in step (c) is from about 300 to 400 psi.

10. A method as in claim 1 wherein the space velocity in step (c) is from about 0.5 to 1.5 vol/vol/hr.

11. A method as in claim 1 wherein the hydrogen dosage is from about 200 to 400 scfb.

12. A method of making transformer oils comprising  
(a) contacting a napthenic oil with air in the presence of a catalyst system comprising a free radical initiating catalyst at a temperature ranging from about 150 to 275° F. and at a pressure ranging from atmospheric to about 300 psi;

(b) fractionally distilling the product of (a); and  
(c) contacting the overhead from (b) with hydrogen in the presence of a hydrogenation catalyst at a temperature from about 550 to 600° F. at a pressure from about 300 to 400 psi at a space velocity ranging from about 0.5 to 1.5 vol/vol/hr at a hydrogen dosage between about 200 to 400 scfb.

\* \* \* \* \*